

## 1

3,437,474

**METHOD OF MAKING ORE AGGLOMERATES**  
Louis George Imperato, Tenafly, N.J., assignor to Blocked  
Iron Corporation, a corporation of New York  
No Drawing, Continuation-in-part of application Ser. No. 5  
374,191, June 10, 1964. This application Oct. 2, 1967,  
Ser. No. 672,003

The portion of the term of the patent subsequent to  
May 7, 1985, has been disclaimed  
Int. Cl. B22b 1/24; B21b 1/28

U.S. Cl. 75—3

8 Claims 10

## ABSTRACT OF THE DISCLOSURE

A method is provided for producing lump metal ores by admixing the finely divided ore with an alkaline earth oxide or hydroxide and a carbonaceous material, forming the mixture into lumps and reacting it with carbon dioxide in the presence of moisture to form alkaline earth carbonates in situ in the lumps.

This application is a continuation in part of my pending application Ser. No. 374,191, filed June 10, 1964, now Patent No. 3,382,063.

This invention relates to ore agglomerates and methods of making the same and particularly to a high strength and at least partially self-reducing iron ore agglomerates and methods of making such agglomerates.

The need for a satisfactory method of agglomerating iron and other ores, particularly oxide ores, has long been recognized. As the high purity, lumpy ores of the Mesabi and other ranges have been exhausted it has been necessary to turn to ore concentrates recovered from less pure ore deposits and to fine ores not heretofore considered suitable for steel making. In order to make these ores suitable for handling and use in steel melting furnaces it has been necessary to agglomerate these ores into larger pieces. This has conventionally been done by pelletizing or briquetting the fine ores and sintering or fusing the pellets or briquettes to form the solidified agglomerates. Sintering requires extremely high temperatures and large capital outlays in temperature resistant equipment.

I have invented an ore agglomerate and method of making such agglomerates which is much less expensive than these sintered agglomerates and is at least partially self-reducing.

In the preferred practice of my invention I admix ore fines with an oxide or hydroxide of an alkaline earth metal, a finely divided carbonaceous material of the group consisting of coal (both bituminous and anthracite), coke, graphite, charcoal, coke breeze and optionally with a small amount of a mineral acid salt of an alkali metal, or an alkaline earth metal and/or a small amount of an alkali hydroxide together with sufficient water to permit the formation of agglomerates such as pellets, briquettes or blocks. These agglomerates are then subjected to an atmosphere of carbon dioxide for a time sufficient to convert a major portion of the alkaline earth oxide or hydroxide to carbonate.

I have found that the moisture level for most effective operation of my process is below 10% by weight of the total admixture and preferably in the neighborhood of 5% or less.

Preferably the carbonaceous material used in my process is finely divided bituminous coal and I shall hereafter discuss the invention in terms of iron ores and bituminous coal. I prefer the size range of 4 mesh and under for the coal used and good results have been attained at both ends of the range as well as with mixtures of varying particle size coal. I have found that amounts between about 1%

## 2

to 15% of coal by weight are most satisfactory for my purposes, although larger amounts up to 25% have been satisfactorily used in practicing my process. I have found that the use of minus 100 mesh coal makes it possible to ball or pelletize conventional "as received" specular hematite concentrate without the addition of reground hematite or without the addition of any other fine ore. Prior to my invention, it had been impossible to form balls or pelletize specular hematite by usual balling or pelletizing methods without regrinding or adding another fine ore. This has been one of the very real problems in the heat indurated types of pellets heretofore made and is a very distinct advantage to be gained by the practice of this invention. I have found that this can be accomplished within the range of coal concentration set out hereinabove, although I prefer to use about 10% minus 100 mesh coal when forming specular hematite balls or pellets.

The amount of alkaline earth oxide or hydroxide, e.g. lime, preferably lies in the range from about 5% to 20% by weight of the admixture.

I prefer to add a small amount (up to about 2%) of a solubilizing agent for calcium and magnesium, as disclosed in my Patent No. 2,996,372, such as a sugar containing material, e.g. blackstrap molasses, glucose, fructose, dextrose, syrups, or the like together with a small amount of a mineral acid salt of an alkali or alkaline earth metal such as calcium chloride in an amount less than about 1%. I may also add a small amount of an alkali metal oxide or hydroxide such as sodium hydroxide, preferably in the range of about 0.1% to about 1.5%.

The practice of my invention produces a resulting product which has high strength after being subjected to elevated temperatures, e.g. 1600°–1900° F., and which shows a high percentage of reduced iron after such heating indicating that the product is self-reducing. Both of these properties are highly sought after and difficult to achieve.

The practice of my invention can perhaps best be explained by reference to the following examples which show the significances of the practice of my invention.

## EXAMPLE I

A series of test were made on pellets produced by balling specular hematite "as received" and reground with high volatile coal and low volatile coal and mixtures of the two types of coal, with lime and with 0.5% blackstrap molasses and 0.4% calcium chloride. The coal was used "as received" in which condition its size was minus 4 mesh and reground to 100 mesh (100 M). The lime was a mono hydrated dolomitic lime powder known in the trade as Ohio Super spray hydrate.

A series of tests to determine the green ball strength and characteristics were performed as follows:

### Drop test

60 A representative sample of twenty carefully sized  $-1\frac{1}{2}$ "  $+1\frac{1}{2}$ " green wet balls are dropped individually from a height of eighteen inches onto a steel plate and the number of consecutive drops required for failure is used to determine an arithmetical average.

### Green ball compression test

65 An identical sample as just previously described is used and a compressive load is applied to individual balls and the load required to fracture is used to determine the arithmetical average.

70 The resulting data appear in Table I.

TABLE I.—GREEN BALL STRENGTHS

| Coal, type                           | Coal, percent | Specular Hematite conc. as rec'd, percent | Specular Hematite conc. reground, percent | Lime, percent | Drop test, drops to failure | Compression, lbs. to failure |
|--------------------------------------|---------------|-------------------------------------------|-------------------------------------------|---------------|-----------------------------|------------------------------|
| None                                 | 71.00         | 24.00                                     | 5.00                                      | 6             | 2.2                         |                              |
| High volatile coal, as rec'd         | 64.10         | 21.30                                     | 5.12                                      | 13            | 3.3                         |                              |
| High volatile coal, as rec'd -100 M. | 67.60         | 22.54                                     | 5.12                                      | 14            | 3.3                         |                              |
| Do                                   | 64.10         | 21.30                                     | 5.12                                      | 16            | 4.1                         |                              |
| Do                                   | 56.96         | 18.96                                     | 5.12                                      | 24            | 3.4                         |                              |
| Do                                   | 52.42         | 17.46                                     | 5.12                                      | 40            | 3.2                         |                              |
| Low volatile coal, as rec'd          | 64.10         | 21.30                                     | 5.12                                      | 16            | 3.1                         |                              |
| Low volatile coal, as rec'd -100 M.  | 64.10         | 21.30                                     | 5.12                                      | 18            | 4.1                         |                              |
| High volatile coal, -100 M.          | 83.88         | None                                      | 5.12                                      | 13            | 3.1                         |                              |
| High volatile coal, -100 M.          | 85.00         | None                                      | 7.00                                      | 19            | 3.6                         |                              |

## EXAMPLE II

The pellets of Example I were treated with carbon dioxide at room temperature to harden and convert the lime to carbonate in situ. These hardened pellets were tested as follows:

## Tumble test

A five pound charge of the completed pellets are tumbled in an A.S.T.M. coke tumbler and the residue remaining on a  $+1\frac{1}{4}$ " screen after 280 revolutions is recorded as a percentage of the original five pounds and noted as the tumble strength index.

## Compression test

A representative sample of twenty  $-1\frac{3}{32}$ "  $+1\frac{1}{32}$ " pellets are drawn and a compressive load is applied to individual pellets and the load required to fracture is used to determine the arithmetical average.

The results of these tests are tabulated in Table II.

TABLE II.—ROOM TEMPERATURE STRENGTH DATA

| Coal, percent | Coals, type                                    | Specular Hematite conc., percent |          | Taconite, percent | Lime Hydrate, percent | Compression test, lbs. | Tumble test, 0/0 $+1\frac{1}{4}$ " 280 Rev. |
|---------------|------------------------------------------------|----------------------------------|----------|-------------------|-----------------------|------------------------|---------------------------------------------|
|               |                                                | Rec'd.                           | Reground |                   |                       |                        |                                             |
| 4.74          | High volatile -100 M.                          | 67.60                            | 22.54    | -----             | 5.12                  | 320                    | 99                                          |
| 9.48          | do                                             | 64.10                            | 21.30    | -----             | 5.12                  | 225                    | 99                                          |
| 18.96         | do                                             | 56.96                            | 18.96    | -----             | 5.12                  | 105                    | 96                                          |
| 25.00         | do                                             | 52.42                            | 17.46    | -----             | 5.12                  | 50                     | 96                                          |
| 9.48          | Low volatile -100 M.                           | 64.10                            | 21.30    | -----             | 5.12                  | 170                    | 99                                          |
| 9.48          | High volatile, as rec'd.                       | 64.10                            | 21.30    | -----             | 5.12                  | 250                    | 99                                          |
| 9.48          | Low volatile, as rec'd.                        | 64.10                            | 21.30    | -----             | 5.12                  | 225                    | 98                                          |
| 10.00         | High volatile -100 M.                          | 84.00                            | 0        | -----             | 6.00                  | 260                    | 98                                          |
| 0             | -----                                          | 93.70                            | 6.30     | -----             | 6.30                  | 343                    | 96                                          |
| 0             | -----                                          | 80.90                            | 9.10     | -----             | 9.10                  | 445                    | -----                                       |
| 5             | High volatile -100 M.                          | 90.00                            | 5.00     | -----             | 5.00                  | 205                    | -----                                       |
| 5             | do                                             | 89.00                            | 6.00     | -----             | 6.00                  | 255                    | 99                                          |
| 5             | do                                             | 88.00                            | 7.00     | -----             | 7.00                  | 323                    | -----                                       |
| 9.48          | 50/50 -100 high volatile/-100 low volatile     | 64.10                            | 21.30    | -----             | 5.12                  | 205                    | 99                                          |
| 9.48          | 50/50 as rec'd, high volatile and low volatile | 64.10                            | 21.30    | -----             | 5.12                  | 240                    | 98                                          |

## EXAMPLE III

## Reduction test

The carbonated pellets of Example II were tested at elevated temperatures and in reducing atmospheres as follows and compared to a commercial taconite heat indurated pellet.

Pellets which had been heated in the above described crucible test are placed in a magnetic field and the degree of attraction is recorded as a qualitative observation.

The results appear in Table III.

TABLE III.—CRUCIBLE TEST DATA

| Coal percent-type              | Specular Hematite conc., percent |          | Taconite, percent | Lime hydrate, percent | Crucible test, load to failure, lbs. |    |    |    |    |    |     |
|--------------------------------|----------------------------------|----------|-------------------|-----------------------|--------------------------------------|----|----|----|----|----|-----|
|                                | Rec'd                            | Reground |                   |                       | 0                                    | 15 | 30 | 45 | 60 | 90 | 210 |
| None                           | 72                               | 23       | -----             | 5.00                  | 410                                  | 23 | 14 | 9  | 8  | 11 | 12  |
| 4.74—high volatile -100 M.     | 67.6                             | 22.54    | -----             | 5.12                  | 320                                  | 30 | 30 | 29 | 29 | 27 |     |
| Heat indurated taconite pellet | -----                            | -----    | -----             | -----                 | 500                                  | 23 | 15 | 16 | 19 | 12 | 18  |
| 9.48—high volatile -100 M.     | 64.1                             | 21.3     | -----             | 5.12                  | 250                                  | 27 | 27 | 24 | 22 | 22 | 19  |
| 9.48—high volatile -100 M.     | 64.1                             | 21.3     | -----             | 5.12                  | 225                                  | 30 | 30 | 30 | 29 | 21 |     |
| Do                             | 34.2                             | 51.20    | -----             | 5.12                  | 180                                  | 30 | 30 | 30 | 30 | 30 | 27  |
| 9.48—low volatile as rec'd.    | 64.1                             | 21.3     | -----             | 5.12                  | -----                                | 30 | 25 | 21 | 20 | 20 | 17  |
| 18.96—high volatile -100 M.    | 56.96                            | 18.96    | -----             | 5.12                  | 105                                  | 30 | 23 | 23 | 17 | 15 | 10  |
| 11.00—high volatile -100 M.    | 83.88                            | -----    | -----             | 5.12                  | 160                                  | 30 | 28 | 23 | 20 | 19 | 12  |
| 13.00—high volatile -100 M.    | 81.88                            | -----    | -----             | 5.12                  | 135                                  | 30 | 30 | 29 | 25 | 22 | 16  |
| None                           | 70.0                             | 23.5     | -----             | 6.50                  | 500                                  | 30 | 26 | 23 | 16 | 19 | 17  |
| 10.00—high volatile -100 M.    | 84.0                             | -----    | -----             | 6.00                  | 170                                  | 30 | 30 | 30 | 30 | 26 | 18  |
| Do                             | 83.0                             | -----    | -----             | 7.00                  | 178                                  | 30 | 30 | 30 | 30 | 28 | 22  |
| None                           | 57.00                            | 38.00    | -----             | 15.00                 | 11                                   | 5  | 8  | 8  | 9  | 9  |     |
| 9.48                           | 51.2                             | 34.2     | -----             | 15.12                 | 5                                    | 5  | 3  | 2  | 2  | 3  | 3   |
| None                           | 60                               | 40       | -----             | 2 None                | 10                                   | 2  | 2  | 2  | 2  | 2  | 2   |

<sup>1</sup> Non-carbonated.

<sup>2</sup> Non-carbonated, 0.75 bentonite.

**EXAMPLE IV**

Pellets were made as in Example II by carbonation substituting taconite concentrates for the specular hematite. These pellets were subject to the same tests as Example III and the data tabulated in Table IV.

5

6 EXAMPLE VII

A series of tests were made on pellets produced by mixing together lime hydrate, specular hematite ore in both the "as received" and the "reground" forms

TABLE IV

| Coal percent-type            | Specular hematite conc., percent |          | Taconite, percent | Lime hydrate, percent | Crucible test—load to failure, lbs. |    |    |    |    |    |    |     |  |  |  |
|------------------------------|----------------------------------|----------|-------------------|-----------------------|-------------------------------------|----|----|----|----|----|----|-----|--|--|--|
|                              |                                  |          |                   |                       | After time in minutes               |    |    |    |    |    |    |     |  |  |  |
|                              | Rec'd                            | Reground |                   |                       | 0                                   | 15 | 30 | 45 | 60 | 90 | 30 | 210 |  |  |  |
| None                         |                                  |          | 93.7              | 6.3                   | 343                                 | 30 | 30 | 30 | 30 | 30 | 30 | 30  |  |  |  |
| 5.00 — high volatile — 100 M |                                  |          | 88.0              | 7.0                   | 323                                 | 50 | 40 | 30 | 30 | 30 | 30 | 30  |  |  |  |
| None                         |                                  |          | 93.28             | 16.72                 | 10                                  | 16 | 25 | 20 | 13 | 13 | 19 |     |  |  |  |
| 9.48 — high volatile — 100 M |                                  |          | 83.80             | 16.72                 | 7                                   | 8  | 7  | 9  | 7  | 6  | 8  | 10  |  |  |  |

<sup>1</sup> Non-carbonated.

### EXAMPLE V

Pellets were made by admixing lime hydrate, coal and or as in Example I. The resulting pellets were subjected to carbon dioxide sufficient to form recrystallized limestone in situ. The carbonated pellets were then divided into two parts, one heated to 1600° F. and the other to 1700° F. in an atmosphere containing carbon monoxide such as would be encountered in a blast furnace or like iron handling furnace. The pellets were removed and analyzed for reduced iron. The results are tabulated in Table V.

as in Example I but substituting various other types of carbonaceous material for coal fines and omitting the molasses and chloride. The resulting pellets were subjected to an atmosphere of carbon dioxide as in Example I to form recrystallized limestone in situ. These hardened pellets were tested as were the pellets in Example II. The results of the tests appear in Table VII.

TABLE V.—CARBONATE BONDED PELLET SUMMARY

| Taconite Concentrate                                                           | Percent Reduction |           |
|--------------------------------------------------------------------------------|-------------------|-----------|
|                                                                                | 1,600° F.         | 1,700° F. |
| 6% Lime Hydrate                                                                | 38.7              | 44.8      |
| 6% Lime Hydrate Plus 5% High Volatile Coal (-100 M)                            | 49.1              | 81.5      |
| Specular Hematite Concentrate                                                  |                   |           |
| 23.5% Reground (-325 M) Specular Hematite Plus 5% Lime Hydrate                 | 39.3              | 45.6      |
| 23% Reground Specular Hematite (-325 M)                                        | 50.6              | 74.1      |
| Plus 5% Lime Hydrate Plus 5% High Volatile Coal                                | 39.8              |           |
| As Received Specular Hematite Plus 5% Lime Hydrate Plus 10% High Volatile Coal | 49.1              | 87.1      |

### EXAMPLE VI

An additional series of pellets were made as in Example V and after removal from the heating furnace at 1600° F. and 1700° F., respectively, were screened to determine the amount above 4 mesh and the amount below 20 mesh. They were then jarred for 15 minutes in a container and again screened. The test results appear in Table VI.

TABLE VII.—ROOM TEMPERATURE STRENGTH DATA  
 Pellet Composition: Specular Hematite as received, 17%; Specular Hematite reground, 70%; Lime Hydrate, 9%; Carbonaceous Materials, various, 4%.

| Carbonaceous Materials,<br>type | Compression<br>test, lbs. | Turnle Test,<br>$0.0 + \frac{1}{4}$<br>280 Rev. |
|---------------------------------|---------------------------|-------------------------------------------------|
| Coke Breeze                     | 161                       | 96                                              |
| Anthraeite                      | 113                       | 89                                              |
| Graphite                        | 119                       | 89                                              |
| Charcoal                        | 173                       | 96                                              |

TABLE VI

| Taconite                                                                                                      | Screen Test From Furnace |       |           |       | Screen Test After Jarring |       |           |       |
|---------------------------------------------------------------------------------------------------------------|--------------------------|-------|-----------|-------|---------------------------|-------|-----------|-------|
|                                                                                                               | 1,600° F.                |       | 1,700° F. |       | 1,600° F.                 |       | 1,700° F. |       |
|                                                                                                               | +4 M                     | -20 M | +4 M      | -20 M | +4 M                      | -20 M | +4 M      | -20 M |
| 6% Lime Hydrate                                                                                               | 96.7                     | 1.67  | 96.9      | 1.48  |                           |       | 43.7      | 51.8  |
| 9% Lime Hydrate                                                                                               | 99.9                     | 0.1   | 99.87     | 0.13  | 77.82                     | 21.96 | 78.23     | 21.62 |
| 12% Lime Hydrate                                                                                              | 99.6                     | 0.3   | 99.5      | 0.2   | 83.9                      | 15.9  | 82.8      | 16.8  |
| 9% Lime Hydrate plus 10% High Volatile Coal (minus 8 M)                                                       | 99.2                     | 0.33  | 97.6      | 0.13  | 80.64                     | 17.30 | 80.09     | 15.0  |
| 9% Lime Hydrate plus 8% High Volatile Coal (minus 8 M) and 2% Low Volatile Coal (minus 8 M)                   | 98.62                    | 0.61  | 99.47     | 0.23  | 81.00                     | 16.98 | 84.17     | 14.24 |
| 9% Lime Hydrate plus 8% High Volatile Coal (minus 8 plus 150 M) and 2% Low Volatile Coal (minus 8 plus 150 M) | 96.69                    | 0.56  | 98.57     | 0.42  | 81.77                     | 14.23 | 78.77     | 17.37 |
| Specular Hematite:                                                                                            |                          |       |           |       |                           |       |           |       |
| 25% Reground (minus 325 M) plus 5% Lime Hydrate plus 15% High Volatile Coal (minus 100 M)                     | 99.60                    | 0.35  | 96.80     | 2.54  | 76.77                     | 20.17 | 57.12     | 36.61 |
| Venezuelan Ore:                                                                                               |                          |       |           |       |                           |       |           |       |
| Plus 4.76 Lime Hydrate                                                                                        | 97.59                    | 0.87  |           |       | 60.43                     | 32.41 |           |       |
| 6% Lime Hydrate+15% High Volatile Coal (minus 100 M)                                                          | 98.0                     | 1.0   | 95.4      | 2.0   | 85.70                     | 11.79 | 84.75     | 12.82 |

## EXAMPLE VIII

Pellets made for Example VII were then treated in the heated furnace as in Examples V and VI. The test results appear in Table VIII.

TABLE VIII  
Pellet Composition: Specular Hematite as received, 17%; Specular Hematite reground, 70%; Lime Hydrate, 9%; Carbonaceous Materials, various, 4%.

| Carbonaceous Materials, types       | Screen Test From Furnace |       |           |       | Screen Test After Jarring |       |           |       |
|-------------------------------------|--------------------------|-------|-----------|-------|---------------------------|-------|-----------|-------|
|                                     | 1,600° F.                |       | 1,700° F. |       | 1,600° F.                 |       | 1,700° F. |       |
|                                     | +4 M                     | -20 M | +4 M      | -20 M | +4 M                      | -20 M | +4 M      | -20 M |
| Coke Breeze.....                    | 99.6                     | 0.30  | -----     | ----- | 74.8                      | 23.5  | -----     | ----- |
| Anthracite.....                     | 99.8                     | 0.19  | -----     | ----- | 73.0                      | 26.2  | -----     | ----- |
| Graphite.....                       | 99.7                     | 0.28  | -----     | ----- | 73.6                      | 24.6  | -----     | ----- |
| Charcoal.....                       | 99.5                     | 0.33  | -----     | ----- | 78.0                      | 21.2  | -----     | ----- |
| Heat, Indurated Taconite Pellet.... | 91.67                    | 1.37  | 93.41     | 1.37  | 72.24                     | 15.35 | 68.17     | 20.03 |

It will be evident from the foregoing tables and examples that a high strength pellet capable of a high level of self-reduction can be achieved by the practice of my invention.

While I have described certain preferred practices and products according to my invention, it will be understood that this invention may be otherwise embodied within the scope of the following claims.

I claim:

1. The method of producing a high strength, self reducing lump ore from finely divided iron containing materials comprising the steps of admixing the finely divided iron containing material with at least one of the group consisting of the oxides and hydroxides of alkaline earth metals and with a carbonaceous material from the group consisting of coal, coke, graphite, coke breeze and charcoal, forming the mixture into lumps and reacting the lumps with carbon dioxide in the presence of moisture to form alkaline earth carbonates in situ in the lumps.

2. The method as claimed in claim 1 wherein up to about 2% by weight of the total mixture of a solubilizing agent for alkaline earth metals is added.

3. The method as claimed in claim 1 wherein a mineral acid salt from the group consisting of alkali and alkaline earth metals is added in an amount up to about 1% on the weight of the admixture.

4. The method of producing a high strength, self reducing lump ore from finely divided metal containing materials comprising the steps of admixing the finely divided metal containing material with at least one of the group consisting of the oxides and hydroxides of alkaline earth metals and with a carbonaceous material from the group consisting of coal, coke, graphite, coke breeze and charcoal, adding thereto up to about 2% of a solubilizing agent for magnesium and calcium, up

to about 1% of mineral acid salt of a member from the group consisting of alkali metals and alkaline earth metals and about 0.1% to about 1.5% of a member from the group consisting of alkali metal oxides and hydroxides,

forming the mixture into lumps and reacting the lumps with carbon dioxide in the presence of moisture to form alkaline earth carbonates in situ in the lumps.

5. The method as claimed in claim 4 wherein the moisture level in the mixture is less than about 10% by weight on the total admixture.

6. The method of producing a high strength, self reducing lump ore from finely divided iron containing materials comprising the steps of admixing the finely divided iron containing material with about 5% to 20% of at least one of the group consisting of the oxides and hydroxides of alkaline earth metals and with between about 1% to 25% of a carbonaceous material from the group consisting of coal, coke, coke breeze, graphite and charcoal, forming the mixture into lumps and reacting the lumps with carbon dioxide in the presence of moisture to form alkaline earth carbonates in situ in the lumps.

7. The method as claimed in claim 6 wherein up to about 2% of a solubilizing agent for calcium and magnesium is incorporated into the admixture.

8. The method of producing a high strength lump iron ore as claimed in claim 6 wherein the mixture contains up to about 10% moisture.

## References Cited

## UNITED STATES PATENTS

|    |           |         |                 |       |      |
|----|-----------|---------|-----------------|-------|------|
| 45 | 145,462   | 12/1873 | Taylor          | ----- | 75—3 |
|    | 2,823,109 | 2/1058  | Sudo            | ----- | 75—3 |
|    | 2,996,372 | 8/1961  | Imperato        | ----- | 75—3 |
|    | 3,205,063 | 9/1965  | Franklin et al. | ----- | 75—3 |

L. DEWAYNE RUTLEDGE, Primary Examiner.

ERNEST L. WEISE, Assistant Examiner.